

## UNITED STATES PATENT OFFICE

1,977,332

METHOD OF FORMING A FUEL  
BRIQUETTECharles Burnet Wood, Los Angeles, Calif., assignor  
to Carbon Products Co., Inc., Los Angeles, Calif.,  
a corporation of CaliforniaNo Drawing. Application March 30, 1932,  
Serial No. 602,108

2 Claims. (Cl. 44—16)

This invention relates to a fuel briquette and the process of making the same.

The fuel briquette about to be described is thought to be novel in several particulars, to-wit: 5 It is possible to ascertain in advance and to so form the briquette that a given result may be accomplished such as, for instance, a complete burning of the briquette without ash or smoke, a burning of the briquette with smoke, or the burning of 10 the briquette with or without smoke with an ash residue. Likewise, the briquette may be formed to burn for a selected duration of time.

An object of the invention is the provision of a fuel briquette which may be stored out of doors 15 without the necessity of covering the same, no deterioration of the briquette being apparent.

Another object is the provision of a fuel briquette which will withstand rough handling without breaking or cracking.

20 Another object is the provision of a briquette which is readily ignited and burns with an even heat.

Another object is the provision of a briquette which may be formed within a minimum of time, 25 to-wit, within a few hours.

Another object is the provision of a briquette which is useful for the heating of orchards and the briquette is adapted to be placed upon the ground without the necessity of confining the 30 same within a container.

Another object is the provision of a briquette which is low in cost of manufacture, does not require expensive apparatus to produce the finished product, which is adaptable for any given fuel 35 requirement, and generally superior to briquettes now in general use so far as the inventor is aware.

With the above and other objects in view, the invention consists in the novel and useful combination of ingredients and method of manufacture, all as disclosed generally in the statement 40 of the invention hereinafter set forth, and more specifically pointed out in the claims.

One important feature of the invention resides in the fact that the fuel briquette of this invention does not require molding under pressure in order to produce a hard briquette. As a matter of fact, actual tests have shown that the briquette of this invention will withstand greater crushing stress than the ordinarily molded briquette. It 50 is, of course, possible to obtain the charcoal of the briquette from various basic materials. For this purpose, any cellulose or carbonaceous material may be used, such as coal, petroleum coke, brush, vegetables, and like materials. Assuming that a 55 material of this character is used, said material

is placed within a suitable crushing or grinding machine, sometimes termed in the industry as a "hogger" so that said material is chopped into fine pieces. After the chopping, the material is placed in an air-tight container and subjected to 60 various heats, although I have found 700° Fahrenheit satisfactory, which heat is maintained for a period of 1½ to 2 hours. The gases are directed from the container and trapped so that by-products may be formed, such as wood alcohol, tannic 65 acids, and various other wood derivatives. After the formation of the charcoal in the manner aforesaid, the charcoal is ground to a selected mesh. In the present instance, we will assume a mesh of 100, which in common parlance means 70 that the particles will pass through a screen having 100 holes to the square inch. In the manner aforesaid, I have produced ground charcoal which will be used as the base material in the formation of the briquette.

I next employ an agitator or a mixer of some type, into which agitator or mixer I place the charcoal together with a binding substance, such as beet, cane sugar or wood syrup which has been thinned with water.

In addition to the foregoing, I add sand to the mix. The addition of the sand is one of the important features of the invention. As an example, I may state that the weight of the binder and sand will vary under given conditions, but if a 85 slow burning briquette is desired, the relative proportions by weight are: ½ charcoal; ¼ sand; and ¼ binding material. After placing the elements just mentioned in the agitator or mixer, the said ingredients are thoroughly mixed and 90 the binder is sufficiently thinned to the end that every particle of the charcoal and sand is contacted. After the various ingredients aforesaid have been thoroughly mixed together, the said ingredients now thoroughly intermixed are poured into molds having any shape desired. The molds are then placed in an evaporating oven to remove all moisture from the briquettes, after 95 which the molds are placed within an oven and subjected to intense heat of approximately 700° 100 Fahrenheit, although other heats may be employed, for a period of approximately 2 hours. After the baking is completed, the briquettes are kept air-tight either by an air-tight mold or covering with sand until the briquettes are thoroughly 105 cold.

I have found that the sugar content of the binding material becomes very hard carbon and that the sand gives an additional strength to the briquette. The sand tends to fuse with the result 110

that the briquette will stand rough handling and not subject to ready breakage. Furthermore, in actual use, the sand does not detract from the heat value of the burning briquette, as the hot sand during the burning throws off radiant rays and aids in the control of even combustion of the carbon content of the briquette.

Voids are, of course, formed in the briquette after its manufacture in accordance with the method aforesaid. These voids enable me to thoroughly impregnate the briquette after it is cool with an inflammable fluid without detracting from the hardness and strength of the briquette. For this purpose, I may use coal oil and paraffin wax, rosin, and the like. Preferably I impregnate the briquette with hot oil and paraffin wax so that upon cooling, the paraffin wax will hold the coal oil within the briquette. I have found in actual practice that hot paraffin will penetrate the briquette within ten to fifteen minutes of time, and has no deleterious effect upon the binder material.

While to begin with, the binder material was soluble in water, yet after the formation of the briquette, the briquette is anhydrous for the reason that the binding material becomes a hard carbon. In place of the coal oil and paraffin wax just mentioned, I may use wood alcohol treated with rosins and soap stock. Obviously, the purpose of the impregnation is to allow a ready igniting of the briquette as the inflammable fluid will generate an intense heat sufficient to ignite the carbon substance.

If I desire the briquette to give off an odor, in place of impregnating the said briquette with an oil, such as coal oil and paraffin, I impregnate the briquette with a powder carried in solution. The solution may be water or other liquid. It is obvious that when the briquette is impregnated with a coal oil and paraffin that a smoke will be given off by the briquette until the paraffin and coal oil are completely burned. However, if in place of coal oil and paraffin I utilize wood alcohol treated with rosins and soap stock as the im-

pregnating substance, the briquette will burn without smoke.

The rapidity with which the briquette is burned is in a measure regulated by varying the solid material.

It is obvious that various changes and modifications and variations may be made in proportions of the various ingredients used in the forming of the briquette, all within the scope of the invention as defined by the scope of the appended claims.

I claim:

1. The method of forming a slow burning hard fuel briquette that withstands great crushing stress adapted for use as an orchard heater, which consists in mixing approximately one-half charcoal, one-fourth sand, and one-fourth a sugar syrup binder, agitating the mix until every particle of the charcoal and sand is coated by the sugar syrup binder, pouring the mixed ingredients into a mold to form a briquette without applying pressure, evaporating the moisture content from said briquette in the mold, subjecting the briquette to a heat of approximately 700° Fahrenheit for a period of about two hours to form an anhydrous porous mass, followed by allowing said briquette to cool under air-tight conditions.

2. The method of forming a slow burning hard fuel briquette that withstands great crushing stress adapted for use as an orchard heater, which consists in mixing approximately one-half charcoal, one-fourth sand, and one-fourth a sugar syrup binder, agitating the mix until every particle of the charcoal and sand is coated by the sugar syrup binder, pouring the mixed ingredients into a mold to form a briquette without applying pressure, evaporating the moisture content from said briquette in the mold, subjecting the briquette to a heat of approximately 700° Fahrenheit for a period of about two hours to form an anhydrous porous mass, followed by allowing said briquette to cool under air-tight conditions, and thereafter impregnating said briquette with a burnable fuel.

CHARLES BURNET WOOD.

80

85

90

95

100

105

110

115

120

125

130

135

140

145

150

45

50

55

60

65

70

75